

# UNITED STATES PATENT OFFICE.

GEORGE T. BLOOM, OF MAGNOLIA, NEW JERSEY.

## COATED WOODEN RECEPTACLE.

1,291,696.

Specification of Letters Patent. Patented Jan. 14, 1919.

No Drawing.

Application filed December 13, 1916. Serial No. 136,757.

To all whom it may concern:

Be it known that I, GEORGE T. BLOOM, a citizen of the United States, residing at Magnolia, in the county of Camden and State of New Jersey, have invented certain new and useful Improvements in Coated Wooden Receptacles, of which the following is a specification.

My invention relates to a process of coating or insulating the surface or interior of containers or receptacles, formed of wood, metal or the like, and which are adapted to receive and hold hydrocarbons, such as oil, gasolene and the like.

15 My process consists generally in applying a suitably concentrated solution of waste sulfite liquor, or sulfite pitch, of acid reaction, to the interior of the container, and allowing the liquid to preferably partly dry, providing a coherent continuous film coating, of desired character.

It has been found that the coating produced by my process is insoluble in hydrocarbons, such as oil, gasolene or the like. A 25 further advantage obtained in connection with my process is that the coherent coating produced thereby is highly soluble in water, thereby allowing the container to be readily cleaned, by the application of hot water or steam.

I am aware of the fact that it is old in the art to coat the interior of containers formed of wood or the like with a solution of glue. This glue coating is not wholly satisfactory, 35 inasmuch as it is soluble in hydrocarbons such as oil, gasolene or the like, producing what is known as "foots" or "sludge." This "foots" is often very injurious or destructive to the hydrocarbons contained in the receptacle. The glue coating renders it difficult to thoroughly clean the receptacle, since the glue, when dried, is not readily soluble in water or steam. It has also been customary to employ a coating comprising a solution of glue mixed with other materials, and the container has also been subjected to several coatings.

I am also aware of the fact that attempts have heretofore been made to utilize the

waste sulfite liquor or sulfite pitch, in coating containers, but such attempts, as far as I am aware, have not proven wholly satisfactory, owing to the use of such material of an improper density. Furthermore, it has been customary to mix with such coating material other coating materials which react with it and prevent the formation of a continuous film. It has also been customary to add neutralizing materials to the sulfite pitch, and these materials have been mixed with the pitch, or applied thereto after the pitch has been coated upon the surface of the container, or coated upon the container, prior to the application of the sulfite pitch thereto. As far as I am aware, these processes require the coating material to be applied while hot.

In the practice of my process, in its preferred form, I employ the waste sulfite liquor or sulfite pitch in a concentrated form, the same having a density of approximately 1.18 specific gravity. This pitch is also in a slightly acid condition. The sulfite pitch may be applied to the surface of the container, which may be a wooden keg 75 or barrel, by spraying, flowing or brushing the same thereon, or in any other suitable manner. I prefer, however, to spray a thin coating of the liquid on the surface of the wood, which wood surface should preferably be dry, whereby I may utilize the absorption of the excess of the moisture by the wood, to bring about partial drying. It is not necessary or desirable that the coating should be completely dried, as partial dryness is preferred, the same producing a film which will stretch rather than crack or break, when subjected to strain.

It is to be understood that the form of my invention herewith shown and described is to be taken as a preferred example of the same, and that various changes may be resorted to in the steps of the process and details of procedure, without departing from the spirit of the invention or the scope of the subjoined claim.

Having thus described my invention, I claim:

A wooden receptacle having its inner surface coated with a partly dried elastic coating, said coating consisting entirely of concentrated waste sulfite liquor or sulfite pitch 5 of a density of approximately 1.18 specific gravity and having an acid reaction which is un-neutralized.

In testimony whereof I affix my signature in presence of two witnesses.

GEORGE T. BLOOM.  
Witnesses:

JAMES C. GOOD,  
EDWARD J. GORMLEY.